

## UNITED STATES PATENT OFFICE

2,439,221

## SILK TREATMENT

Ben W. Rowland and Douglas Fronmuller, Appleton, Wis., assignors to The Institute of Paper Chemistry, Appleton, Wis., a corporation of Wisconsin

No Drawing. Application June 14, 1940,  
Serial No. 340,573

1 Claim. (Cl. 117—139.5)

1

The present invention relates generally to the treatment of silk and more specifically to the step in the processing of silk known in the art as the throwing operation.

The principal object of the present invention is to provide silk processing treatments which serve as practical means for obtaining improved silk.

Other objects will be apparent as the description hereinafter proceeds.

Heretofore, in processing silk for use in the art as, for example, in the manufacture of silk hosiery, it has been customary practice to carry out all chemical processing treatments in alkaline baths. An illustrative example is the throwing bath used in the throwing operation, i. e., a processing step employed to loosen up and soften the individual strands of raw silk to the extent that the skein of silk can be reeled off onto a reel prior to twisting and coning. The silk obtained after treatment in such baths (particularly the throwing bath where the silk remains in contact with the alkali for some time) has long been recognized by the art as relatively unsatisfactory.

We discovered after an extended investigation that acid throwing baths having pH values between 3 to 5.8 and preferably around 3.45 provide practical means for obtaining improved silk. For example, hosiery made from the silk processed in the acid baths of the present invention, has improved stretch and tensile strength characteristics, improved form-fitting, e. g. less slackening at the knees after a period of wear, and exhibits a definitely cleaner knitting stitch.

The throwing baths are aqueous baths containing small amounts of (1) a softening oil such as mineral oil, cocoanut oil, etc., in emulsified form, and (2) an acidic material such as glyceryl lauryl sulphate, acetic acid, etc. The preferred baths also contain a penetrating agent such as a surface-active alkali metal sulphate or sulphonate or a phospholipid such as lecithin. Materials of this type in addition to penetrating action may aid in the emulsification of the oil as well as serve as acidic buffers. The following representative baths or throwing emulsions will serve for illustrative purposes.

*Emulsion 1*

A bath composed of about 100 parts of water, about 0.5 part of the sodium salt of monoglyceryl lauryl sulphate, about 2.5 parts of mineral oil and sufficient monoglyceryl-lauryl sulphate to adjust the pH of the mixture to about 3.45. In this emulsion the ingredients are added in the usual man-

5  
15

2

ner and after mixing the bath is stirred vigorously, or passed through a colloid mill in order to emulsify the oil.

*Emulsion 2*

A bath composed of about 200 parts of water, about 10 parts of lecithin oil and sufficient acetic acid buffered by sodium acetate to adjust the pH of the mixture to a range of about 3.0 to 5.5. In this emulsion the acidic material is preferably added after the water and lecithin oil have been heated, e. g. to 50°-60° C. and stirred vigorously in order to emulsify the oil. The lecithin oil referred to herein is a crude lecithin composition containing about 40 to 60 per cent cocoanut oil.

*Emulsion 3*

A bath composed of about 200 parts water, about 5 parts lecithin, about 5 parts mineral oil and sufficient acidic material such as acetic acid containing a buffer such as sodium acetate to adjust the pH of the mixture to a range of about 3.0 to 5.5. In this emulsion the ingredients may be added in the usual manner and the bath stirred vigorously in order to emulsify the oil in accordance with the above examples.

*Emulsion 4*

A bath composed of about 100 parts water, 0.5 part of the sodium salt of monoglyceryl-lauryl sulphate, 1.25 parts mineral oil, 1.25 parts of 50 per cent sulphonated castor oil, and sufficient acetic acid to adjust the pH of the mixture to 3.45. This mixture is agitated sufficiently in the usual manner to form a stable emulsion consisting of small drop sizes.

It will be understood that the present invention is not limited to the above illustrative examples. For example, in place of the oils listed above other softening oils may be employed, although the use of a relatively inert aliphatic oil is generally preferred. In place of glyceryl lauryl sulphate, other materials such as sulphated cottonseed oil, sulphonated castor oil (Turkey red oil), oleyl sulphate and an alkyl aryl sulphate sold in the trade as "Nacconal" may be used if desired. In place of acetic acid, other acidic materials such as citric acid may be employed. The acidic material in any event should be present in sufficient amount to adjust and maintain the pH value to approximately 3.0-3.3 to 5.5-5.8.

The following comparative tests results obtained with silk processed in (1) the standard alkaline throwing bath and (2) the new acid throwing bath will serve to illustrate the im-

50  
45  
55

Improvements obtainable by processing silk in accordance with the present invention.

Table I

|                       | Alkaline Thrown Silk   | Acid Thrown Silk       |
|-----------------------|------------------------|------------------------|
| Stretch.....          | 1.0 in. per 10 in..... | 2.0 in. per 10 in..... |
| Tensile Strength..... | 176.5 grams.....       | 212 grams.....         |

The above tests were carried out after coning on a Scott inclined plane tester. The tests results which are representative show a 100 per cent increase in stretch and about a 20 per cent improvement in tensile strength.

Table II

|                                    | Alkaline Thrown Silk | Acid Thrown Silk |
|------------------------------------|----------------------|------------------|
| Variation on a 30 inch length..... | 1.0 in.....          | 0.25 in.....     |

The above tests were carried out after knitting on commercial equipment, the alkaline and acid thrown silks being run side by side in the same room (under the same conditions, e. g. humidity, etc.) on the same machine bank. The measurements were made on the length of the legs of the knitted hosiery.

Table III

|                                 | Alkaline Thrown Silk | Acid Thrown Silk |
|---------------------------------|----------------------|------------------|
| Average Wearing Life Ratio..... | 200 hours.....       | 600 hours.....   |

The above tests were carried out on silk stockings after the usual alkaline-soap "boil off," i. e. removal of silk waxes, and dyeing operation. The stockings made from acid thrown silk in addition to the remarkable increase in wearing life also exhibited improved washability.

Our investigations indicate that the throwing operation i. e. treatment of the silk, should be carried out in the acid baths of the present invention at about 70°-100° F. for about 10 to 30 minutes. Ordinarily a temperature of about 80° F. is preferred and a treatment or soaking period of about 15 minutes adequate, as our investigation shows that the silk takes up the available oil much more readily in the acid baths of the present invention than in the standard alkaline throwing baths employed heretofore. Comparative measurements, for example, have

been made on the oil pickup in throwing baths containing the same amount of available oil and it was found that 94 per cent of the available oil was taken up in an acid bath in a given period while only 31 per cent of the available oil was taken up in the same period in an alkaline bath.

The throwing operation of the present invention may be carried out on raw silk, although it is preferred to practice the process of the present invention in combination with the preliminary acid rinse process described and claimed in our copending application Serial No. 340,572, now abandoned. Such a combined process includes (1) an initial treatment of raw silk with a bath having a pH value of 3.5 to 5.5 and consisting of water, acidic material and a buffer, i. e. in the absence of oil, and (2) followed by an acidic throwing treatment in the presence of oil as herein described.

It will be understood that the present invention is not limited to the above illustrative examples. All modifications coming within the scope of the present invention are intended to be covered by the following claim.

25 We claim:

In the art of processing silk, the improvement which comprises subjecting silk to a treatment in an aqueous bath consisting of a mineral oil emulsion, a small amount of the sodium salt of monoglyceryl-lauryl sulphate, a small amount of sulphonated castor oil and sufficient acetic acid to adjust the pH value of said bath to about 3.45.

BEN W. ROWLAND.  
DOUGLAS FRONMULLER.

## REFERENCES CITED

The following references are of record in the file of this patent:

## UNITED STATES PATENTS

| Number    | Name        | Date          |
|-----------|-------------|---------------|
| 354,223   | Randall     | Dec. 14, 1886 |
| 1,491,228 | Genstein    | Apr. 22, 1924 |
| 1,865,897 | Gilligan    | July 5, 1932  |
| 2,012,610 | Lenher      | Aug. 27, 1935 |
| 2,023,387 | Harris      | Dec. 3, 1935  |
| 2,025,989 | Kaplan      | Dec. 31, 1935 |
| 2,029,969 | Wallerstein | Feb. 4, 1936  |
| 2,067,888 | Chamberlin  | Jan. 19, 1937 |

## OTHER REFERENCES

Textile Research, Cambridge, 1932, U. S. Institute for Textile Research, pages 157, 167.

La Motte: The ABC of Hydrogen Ion Control, 5th ed., Baltimore, 1929, pages 45 and 46.